

# UNITED STATES PATENT OFFICE.

PETER SOUDERS, CHESTER SMITH, HORACE MILTON CRAIGHEAD, AND  
NORTON SOUDERS, OF RIEGLESVILLE, NEW JERSEY.

## BLEACHING COMPOUND FOR JUTE PAPER-STOCK, &c.

SPECIFICATION forming part of Letters Patent No. 312,525, dated February 17, 1885.

Application filed September 22, 1884. (Specimens.)

*To all whom it may concern:*

Be it known that we, PETER SOUDERS, CHESTER SMITH, HORACE M. CRAIGHEAD, and NORTON SOUDERS, citizens of the United States, residing at Rieglesville, in the county of Hunterdon, and State of New Jersey, have invented certain new and useful Improvements in Bleaching Compounds for Jute Paper-Stock, &c.; and we do declare the following to be a full, clear, and exact description of the invention, such as will enable others skilled in the art to which it appertains to make and use the same.

This invention has relation to bleaching jute paper-stock; and it consists in the process hereinafter set forth, and pointed out in the appended claim.

In carrying out this process the jute-stock is first thoroughly washed in the usual manner. Then a composition of ten pounds of alum, four pounds of South Carolina clay, and two gallons of water is boiled and added to five hundred pounds of the stock, which is then run in the mixing-engine for fifteen minutes, after which fifty pounds of bleaching-powder are added. In like proportion the composition and bleaching-powder are used with larger amounts of the stock, so that one-half of the bleaching-powder used in the processes heretofore employed is saved, as it has required one hundred pounds of bleaching-pow-

der to bleach five hundred pounds of this stock.

Resulting from this process it is designed to produce a paper of better color and greater strength, and the manufacture is cheapened and facilitated, not only by lessening the quantity of bleaching-powder, but by avoiding to a great extent the annoyance of foam and the use of coal-oil in killing the same. It also saves the wire-cloth jacketing and the felts used on the paper-machines.

Having described this invention, what we claim, and desire to secure by Letters Patent, is—

The process of bleaching jute paper-stock which consists in mixing with the stock a composition of alum and clay raised to steam-heat, and afterward adding a quantity of bleaching-powder, in the proportion and manner substantially as set forth.

In testimony whereof we affix our signatures in presence of two witnesses.

<sup>his</sup>  
PETER X SOUDERS.  
mark.

CHESTER SMITH.  
HORACE MILTON CRAIGHEAD.  
NORTON SOUDERS.

Witnesses:

THOMAS NEWMAN,  
CHS. F. FITCH.